

3,523,796  
DEVELOPMENT OF LIGHT-SENSITIVE  
SILVER HALIDE EMULSIONS

Jozef Frans Willems, Wilrijk, Francis Jeanne Sels, Kontich, and Robrecht Julius Thiers, Brasschaat, Belgium, assignors to Gevaert-Agfa N.V., Mortsel, Belgium, a company of Belgium  
No Drawing. Filed Aug. 9, 1967, Ser. No. 659,334  
Claims priority, application Great Britain, Aug. 30, 1966, 38,552/66

Int. Cl. G03c 5/30

U.S. Cl. 96—66

4 Claims

### ABSTRACT OF THE DISCLOSURE

Photographic light-sensitive silver halide materials comprising a polymeric compound containing N-alkyl-alkylene-amino groups in base or salt form linked through hydroxy-substituted oxyalkylene groups are described. The polymeric compounds in the silver halide materials increase the developability and sensitivity of the photographic emulsion.

This invention relates to a process for producing a photographic silver image by development of exposed light-sensitive silver halide in the presence of compounds influencing the sensitometric characteristics of a light-sensitive silver halide emulsion by an increase of the speed and/or the gradation. The present invention also relates to said compounds used in said process, their preparation and to photographic materials and developing baths containing said compounds.

It is known that the general sensitivity of photographic emulsions, which can already be sensitized optimally throughout the whole range of the spectrum by means of the so-called chemical sensitizers, such as sulphur sensitizers, can be increased if amines or some polyamines such as diethylenetriamine, triethylene-tetramine, are added to these photographic emulsions (British specification 734,474 filed Nov. 6, 1953, by Kodak). Such substances, however, cause an increase of the free silver ion



concentration of the emulsion and greatly diminish its stability.

It is also known that an increase of sensitivity can be obtained by incorporating into the photographic material polyethylene glycols, alkylene oxide polymers obtained by polymerising alkylene oxide in the presence of hexitol ring dehydration products, aliphatic alcohols, aliphatic acids, amines, amides, and phenols (British specifications Nos. 548,019, filed Mar. 19, 1941, by Kodak; 600,058, filed Jan. 10, 1946, by Du Pont de Nemours; 592,676, filed Apr. 20, 1945, by Du Pont de Nemours; 748,745, and 748,750, both filed June 28, 1954, by Kodak).

It is further known that these polyglycols and alkylene oxide polymers should possess a molecular weight of at least 400. In order to obtain a noticeable effect, it is in practice necessary to use compounds having a molecular weight of 1500 to 2000 and more.

Contrary to the other known methods for increasing the sensitivity of silver halide emulsions such as those in which the chemical sensitizers increase the inherent sensitivity and those in which the cyanine dyes increase the spectral absorption, it appears that the final sensitivity of the silver halide emulsion layers in which these compounds are incorporated is higher since these compounds exert a favourable influence on the development of these

silver halide layers by means of the usual developers. Consequently these compounds can be considered as development accelerators.

It is also known, however, that a noticeable increase in sensitivity is only obtained with these compounds when developing in rather slow working developers of the fine grain developer type used in the development of continuous tone images. In fast acting p-N-methyl-aminophenol hydroquinone or 1-phenyl-3-pyrazolidinone hydroquinone developers, their development accelerating action manifests itself only by a very moderate increase of the speed of the developed photographic material.

It is further known that these compounds when used in silver halide emulsion layers of the more sensitive type impair the keeping qualities of these layers, particularly at high temperatures and elevated degrees of relative humidity, since they induce a substantial increase of fog. It also has been observed that the incorporation of these compounds into the photographic material in order to prepare more sensitive silver halide emulsion layers impairs the image tone of the developed silver, thereby forming brown and reddish brown images.

It has been found now that polymeric compounds containing N-alkyl-alkylene-amino groups in base or salt form linked through hydroxy-substituted oxyalkylene groups and such polymeric compounds wherein the hydrogen atoms of the said hydroxy groups are partly or wholly substituted, are very suitable for substantially increasing the developability and also the sensitivity of photographic silver halide emulsion layers on development in slow as well as in fast acting developers, and practically do not impair the keeping qualities of the said layers.

Polymers, which have proved to be very suitable in that respect, contain structural units which are represented by the following structural Formulae A and B:



wherein:

R represents a C<sub>1</sub>—C<sub>5</sub> alkyl group including a substituted C<sub>1</sub>—C<sub>5</sub> alkyl group, e.g., methyl, ethyl, propyl, isopropyl or 2-hydroxyethyl, or an aralkyl group, e.g., benzyl, each of Alk<sub>1</sub> and Alk<sub>2</sub> represents an alkylene group containing from 2 to 10 carbon atoms, including such group substituted by, e.g., a hydroxyl group and/or such group the carbon chain of which is interrupted by hetero atoms, e.g., oxygen, sulphur, phosphorus, or a substituted nitrogen atom such as an alkyl-substituted nitrogen atom,

n is a positive integer of at least 3, and

60 R<sub>1</sub> represents a hydrogen atom, an alkyl group including a substituted alkyl group, e.g., an ethylenenitrile group,



65 where R<sub>2</sub> represents an alkyl group, a monovalent unsaturated aliphatic group such as an alkenyl group, an aryl group or a heterocyclic group including said groups in substituted form.

70 The compounds according to the invention can be prepared by reaction of a monoalkyl-hydroxyalkylene-amine and/or di(hydroxyalkylene)-amine with a bis-epoxide.

The polyaddition is carried out in such a way that the polyaddition products either in the form of the base or in the salt form are soluble in water.

If the reaction between the secondary amine alkanol and the bis-epoxide is too exothermic, care must be taken that the reaction mixture is cooled in order to prevent the formation of gummy products. The optimum reaction temperature is adapted to each polyaddition and usually varies between 50 and 180° C.

When very reactive starting compounds are used, it is sometimes advantageous to mix the reaction products with water at the stage at which the required degree of polyaddition is attained, so that any further addition, which would lead to the formation of water-insoluble products, is prevented. Normally, polymers containing both types of structural units A and B are formed but depending on

1 mole of a secondary amine alkanol is preheated at a temperature comprised between 25 and 130° C. (see Table 1), and subsequently 1 mole of a bis-epoxide is added thereto portion-wise whilst stirring. The addition of the bis-epoxide is regulated so that no gummy products are formed; if necessary the mixture is cooled during the addition. After the addition of the bis-epoxide, the reaction mixture is allowed to react further (see Table 1) in order to obtain products with a higher molecular weight. Care should be taken, however, that the reaction is stopped when formation of water-insoluble gummy products begins. With very reactive starting products it is sometimes necessary to add water to the reaction mixture after the addition of the bis-epoxide to avoid gum formation.

In Table 1 hereinafter a survey of suitable starting products and reaction conditions is given.

TABLE 1

| Compound No. | Used secondary amine alkanol                                 | Used epoxide | Reaction time | Reaction temp. (°C.) | Remarks                                         |
|--------------|--------------------------------------------------------------|--------------|---------------|----------------------|-------------------------------------------------|
| 1.....       | H <sub>3</sub> C—NH—CH <sub>2</sub> CH <sub>2</sub> OH       |              | 2 h. 30'....  | 70                   | Water-soluble viscous mass.                     |
| 2.....       | H <sub>3</sub> C<br>CH—NH—CH <sub>2</sub> CH <sub>2</sub> OH |              | 21 h.....     | 100-130              | Viscous mass, soluble in water/ethanol (50/50). |
| 3.....       | H <sub>3</sub> C<br>CH—NH—CH <sub>2</sub> CH <sub>2</sub> OH |              | 26 h.....     | 100-120              | Idem.                                           |
| 4.....       | H <sub>3</sub> C<br>CH—NH—CH <sub>2</sub> CH <sub>2</sub> OH |              | 50 h.....     | 100-130              | Water-soluble viscous mass.                     |
| 5.....       | H <sub>3</sub> C—NH—CH <sub>2</sub> CH <sub>2</sub> OH       |              | 28 h.....     | 100-120              | Idem.                                           |
| 6.....       | HN—(CH <sub>2</sub> CH <sub>2</sub> OH) <sub>2</sub>         |              | 3 h.....      | 100                  | Idem.                                           |

the reactivity of the respective hydroxyl and secondary amino groups one of both units will dominate in the structure of the polymer.

In general, the starting products are made to react in an equimolar ratio, though an excess of one of them is not harmful in most cases, except in a polyaddition reaction between very reactive compounds, in which an excess of bis-epoxide should be avoided always in order to prevent the formation of polyaddition products, which either in the form of a base or a salt are insoluble in water. Bis-epoxides suitable for use are, e.g., 1,2:5,6-diepoxy-hexane, bis(2,3-epoxypropyl)ether, 1,2 - bis(2,3 - epoxypropoxy)-ethane, 1,3-bis(2,3-epoxypropoxy)-propane, 1,4-bis(2,3-epoxypropoxy) - butane, 1,3 - bis(2,3 - epoxypropoxy)-2-propanol, 1,3-bis(2,3-epoxypropoxy)-butane, 2,3:2',3'-di-epoxy-N-alkyl-dipropylamine, 5,6-epoxy-hexane carboxylic acid-2,3-epoxypropyl ester, bis(2,3-epoxypropyl)-sulphone.

Tri-epoxides such as tri(2,3-epoxypropoxy)-phosphate and 2,4,6-tri(2,3-epoxypropoxy)-s-triazine can also be used.

Particularly suitable secondary amine alkanols are N-alkyl-ethanolamines such as methyl-, ethyl-, propyl-, isopropyl-, and butyl-ethanolamines, N-alkyl-propanolamines, e.g., N-methylisopropanolamine, N- $\alpha$ -methylbenzylethanolamine, etc.

As an illustration of the preparation of said polyaddition products a general procedure of preparation is given hereinafter.

In the preparation of condensation products according to the present invention wherein the hydrogen atoms of the free hydroxyl groups are partly or wholly substituted reagents of the type of those reacting with an active hydrogen atom are used, e.g., an acid chloride or acid anhydride such as acetic anhydride, succinic anhydride, or maleic anhydride, a sulfonyl chloride, an isocyanate or an unsaturated alkylating compound, e.g., a vinyl compound such as acrylonitrile and methacrylonitrile. The reaction product of the hydroxyl-containing polymer with maleic anhydride is preferably allowed to react with a bisulphite thus forming a bisulphite addition product. The bisulphite used is preferably an alkali metal bisulphite. The bisulphite addition compounds applied in the present invention are very less fog-producing and are therefore preferred for being incorporated into the light-sensitive material. The preparations of the compounds 7 to 12 are given to illustrate these reactions.

## COMPOUND 7

To a solution of 24.6 g. (0.1 mole) of compound 5 in 200 ccs. of dioxan, a solution of 19.6 g. (0.2 mole) of maleic anhydride in 150 ccs. of dioxan is dropwise added at reflux temperature in  $\frac{1}{2}$  hr. An oily precipitate is formed and refluxing is continued for 4 hrs. whilst stirring. The dioxan is then decanted from the viscous oil, which is extracted several times with warm dioxan and thoroughly kneaded with ether. The residue is dried

at 60° C. The product obtained is fatty and water soluble. Yield: 39.5 g.

#### COMPOUND 8

To a solution of 13.7 g. (0.05 mole) of compound 3 in 100 ccs. of dioxan, a solution of 9.8 g. (0.1 mole) of maleic anhydride in 50 ccs. of dioxan is dropwise added at reflux temperature in 15 min. An oily precipitate is obtained and refluxing is continued for 4 hours whilst stirring. The dioxan is then decanted from the viscous oil, which is extracted several times with warm dioxan and thoroughly kneaded with ether. The residue is dried at 60° C. The product obtained is fatty and water-soluble. Yield: 23.5 g.

#### COMPOUND 9

To a solution of 13.85 g. (0.05 mole) of compound 4 in 100 ccs. of dioxan, a solution of 9.8 g. (0.1 mole) of maleic anhydride in 50 ccs. of dioxan is dropwise added at reflux temperature in 15 min. An oily precipitate is obtained and refluxing is continued for 3 hours whilst stirring. The dioxan is then decanted from the viscous oil, which is extracted several times with warm dioxan and thoroughly kneaded with ether. The residue is dried at 60° C. The product obtained is fatty and soluble in dilute sodium hydroxide solution. Yield: 20 g.

#### COMPOUND 10

To a solution of 20 g. (0.2 mole) succinic anhydride in 150 ccs. of tetrahydrothiophene-1,1-dioxide, a solution of 27.7 g. (0.1 mole) of compound 4 in 100 ccs. of tetrahydrothiophene-1,1-dioxide is dropwise added at 100° C. in 30 min. Heating is continued for 3 hrs. whilst stirring. The solution is then poured into a mixture of ether and aceton (1000 ccs./300 ccs.) and a viscous oil is obtained which thereafter is still three times kneaded with the same mixture. The residue is dried in a drying oven at 60° C. The product obtained is a water-soluble resin. Yield: 47 g.

#### COMPOUND 11

To a suspension of 23.6 g. (0.05 mole) of compound 9 in 200 ccs. of water, 10.4 g. (0.1 mole) of sodium bisulfite in 100 ccs. of water are dropwise added at room temperature. The mixture is then refluxed for 5 hrs. whereby a solution is obtained. The solution is filtered off, evaporated and dried in the drying oven at 70° C. The product obtained is a water-soluble resin. Yield: 33.5 g.

#### COMPOUND 12

To a solution of 11 g. (0.025 mole) of compound 7 in 100 ccs. of water, 5.2 g. (0.05 mole) of sodium bisulfite in 50 ccs. of water are dropwise added at room temperature. The mixture is refluxed for 5 hrs. and the solution is filtered, evaporated and dried at 70° C. The product obtained is a water-soluble resin. Yield: 14.5 g.

The development accelerators used according to the present invention can be added as a base or in the salt form to the coating composition of a silver halide emulsion and/or incorporated into a water-permeable layer, which applied under or on top of the emulsion layer forms a water-permeable system with the silver halide emulsion layer and thus can come into effective contact with the silver halide.

The development accelerators can be incorporated into the coated emulsion layer either by treating the emulsion layer with an aqueous solution of these development accelerators or by coating this layer with a water-permeable layer containing the development accelerators, or also by bringing the development accelerators from a water-permeable layer lying under the emulsion layer and comprising said development accelerators, by diffusion into effective contact with the silver halide.

The water-soluble development accelerators can be added to the light-sensitive silver halide emulsion during different preparation steps of the light-sensitive material:

for instance they can be incorporated therein as a separate addition either mixed with one or more ingredients, which are used in the preparation of the silver halide grains during the physical or chemical ripening process, or another moment preceding the application of the emulsion.

5 The development accelerators are preferably added to the silver halide emulsion composition after the chemical ripening process and just before coating the emulsion.

10 The development accelerators are preferably added in dissolved form in water or in an aqueous mixture of water and water-miscible organic solvents that do not impair the photographic properties of the light-sensitive silver halide emulsion. When the polyaddition products are not sufficiently soluble in water in their base form, 15 they are converted into their salt form by neutralization, e.g., with an acid such as sulphuric acid, hydrochloric acid, p-toluenesulphonic acid, or acetic acid.

15 The optimum amount of development accelerator added to the silver halide emulsion depends on the very 20 compound, on the nature of the colloid binding agent for the silver halide grains, and on the amount and the kind of the silver halide in the emulsion. In general, however, the development accelerators are added to the light-sensitive material in amounts ranging from 100 mg. to 25 10 g. per mole of silver halide. In the developing bath they are normally used in amounts ranging from 0.1 g. to 10 g. per liter. If necessary, these compounds can also be added in amounts exceeding these limits.

25 The step of increasing the sensitivity according to the 30 present invention can be combined with a method known as chemical sensitisation, in which together with the above-mentioned development accelerators usual amounts of chemical sensitizers are added to the silver halide emulsion, e.g., sulphur-containing compounds such as allyl isothiocyanate, allylthiourea or sodium thiosulphate, reducing compounds such as the tin compounds described in our Belgian patent specifications 493,464, filed Jan. 24, 1950, and 568,687, filed June 18, 1958, both by Gevaert Photo-Producten N.V., the iminoaminomethane sulphonic acid compounds described in the British patent specification 789,823, filed Apr. 29, 1955, by Gevaert Photo-Producten N.V., or noble metal compounds such as gold, platinum, palladium, iridium, ruthenium, and rhodium compounds. As a matter of fact, the sensitising action of the development accelerators used in the present invention comes in addition to the sensitising action of the sensitising compounds originally present in gelatin.

35 The development accelerators applied in the present invention can also be used in combination with stabilisers 40 and fog-inhibiting compounds for the silver halide emulsion, for instance with mercury compounds or organic sulphur-containing compounds that form an insoluble silver salt with silver ions, preferably heterocyclic nitrogen-containing thioxo compounds such as benzothiazolin-2-thione and 1-phenyl-tetrazolin-5-thione, the compounds described in our Belgian patent specifications 571,916 and 571,917, both filed Oct. 10, 1958, by Gevaert Photo-Producten N.V., and compounds of the oxytriazolopyrimidine type, e.g., 5-methyl-7-hydroxy-s-triazolo[1,5-a] 45 pyrimidine. The combination with sensitising and stabilising cadmium salts in the light-sensitive material as well as in the developing bath can also be applied.

50 Other compounds, which sensitise the photographic emulsion by development acceleration, such as organic onium compounds and polonium compounds, preferably of the ammonium or sulphonium type, e.g., quaternary tetra-alkylammonium salts, alkylpyridinium salts, bis-alkylene-pyridinium salts, alkylquinolinine salts and tri-alkyl-sulphonium salts can be used together with the development-accelerators according to the invention in the developing solution as well as in the light-sensitive material. Other ingredients, such as colour couplers, developing substances, hardening agents, and wetting agents, can 55 also be added to the emulsion in the ordinary way.

The development of low-sensitive as well as of high-sensitive, of fine-grain as well as of coarse-grain silver halide emulsions is accelerated by the action of the above-mentioned development accelerators. These products can be applied for accelerating the development of X-ray emulsions as well as of the most different spectrally or nonspectrally sensitised emulsions. They can be incorporated into the photographic emulsion either with or without optical sensitizers and can be used for increasing the sensitivity of negative emulsions as well as of positive emulsions.

The following examples illustrate the invention.

#### EXAMPLE 1

A washed negative gelatin silver bromo-iodide emulsion (average grain size of the silver halide,  $0.8\mu$ ), the silver halide of which consists of 94.5 mole percent of silver bromide and 5.5 mole percent of silver iodide, is ripened at  $45^\circ$  C. The emulsion ready for coating contains per kg. 50 g. of silver halide, 75 g. of gelatin, 30 mg. of optical sensitizer according to the following structural formula:



50 mg. of 5-methyl-7-hydroxy-s-triazolo[1,5-a]pyrimidine as a stabiliser, and 500 mg. of saponine as a wetting agent.

This emulsion is divided into several aliquot portions and to the separate portions is added one of the development accelerators according to the present invention. The emulsion portions are separately applied to a cellulose triacetate support and dried.

The test strips obtained are then exposed in the same conditions through a grey wedge and developed for 7 minutes at  $20^\circ$  C. in a fine-grain developer of the following composition:

Water—800 ccs.  
Monomethyl-p-aminophenol sulphate—2 g.  
Hydroquinone—5 g.  
Anhydrous sodium sulphite—100 g.  
Borax—10 g.  
Boric acid—5 g.  
Potassium bromide—0.5 g.  
Water to—1000 ccs.

The speed is given in exposure values which have to be compared with the exposure value of an emulsion to which no sensitizer was added. A decrease of the exposure value by 30 means a doubling of the speed.

| Number of the added compound | Amount of compound per kg. of emulsion (g.) | Sensitometric results |       |       |
|------------------------------|---------------------------------------------|-----------------------|-------|-------|
|                              |                                             | Fog                   | Gamma | Speed |
| 1                            | 1                                           | 0.05                  | 0.53  | 124   |
| 6                            | 1                                           | 0.07                  | 0.63  | 93    |
| 11                           | 1                                           | 0.07                  | 0.61  | 95    |
|                              |                                             |                       |       | 96    |

#### EXAMPLE 2

Example 1 was repeated but the emulsions contained the development accelerators listed in the following table.

Before development the emulsion strips were conditioned for 36 hr. at  $57^\circ$  C. in an atmosphere of 34 percent relative humidity.

| Added compound                                           | Amount of compound per kg. of emulsion (mg.) | Sensitometric results |       |       |
|----------------------------------------------------------|----------------------------------------------|-----------------------|-------|-------|
|                                                          |                                              | Fog                   | Gamma | Speed |
| Polyethylene glycol with average molecular weight 6,000. | 100                                          | 0.08                  | 0.52  | 124   |
|                                                          |                                              | 0.50                  | 0.53  | 114   |
| 11                                                       | 100                                          | 0.11                  | 0.59  | 99    |

#### EXAMPLE 3

An emulsion as described in Example 1 is used, except that the test strips after having been exposed, are developed for 7 min. at  $20^\circ$  C. in a classical fast acting hydroquinone p-N-methylaminophenol developer of the following composition:

Water—800 ccs.  
p-N-methylaminophenol hemisulphate—2 g.  
Hydroquinone—5 g.  
10 Anhydrous sodium sulphite—25 g.  
Crystalline sodium carbonate—40 g.  
Potassium bromide—1 g.  
Water to—1000 ccs.

15 The sensitometric results are listed in the table hereinafter.

| 20 | Added compound | Amount of compound added per kg. emulsion | Sensitometric results |       |       |
|----|----------------|-------------------------------------------|-----------------------|-------|-------|
|    |                |                                           | Fog                   | Gamma | Speed |
| 1  | 1 g.           |                                           | 0.08                  | 0.31  | 181   |
| 2  | 1 g.           |                                           | 0.05                  | 0.33  | 170   |
| 6  | 30 mg.         |                                           | 0.10                  | 0.41  | 146   |
| 6  | 1 g.           |                                           | 0.04                  | 0.44  | 155   |
| 25 |                |                                           | 0.04                  | 0.39  | 142   |

#### EXAMPLE 4

An emulsion as described in Example 1 is used, except that the test strips after having been exposed, are developed for 8 min. at  $20^\circ$  C. in a developer having the following composition:

N-methyl-p-aminophenol sulphate—4.5 g.  
Sodium sulphite, anhydrous—100 g.  
35 Boric acid—2.2 g.  
Sodium chloride—15 g.  
Water to—1000 ccs.

The sensitometric results are listed in the table hereinafter.

| 40 | Added compound | Amount of compound added per kg. emulsion | Sensitometric results |       |       |
|----|----------------|-------------------------------------------|-----------------------|-------|-------|
|    |                |                                           | Fog                   | Gamma | Speed |
| 2  | 300 mg.        |                                           | 0.07                  | 0.52  | 186   |
| 3  | 300 mg.        |                                           | 0.09                  | 0.50  | 162   |
| 4  | 300 mg.        |                                           | 0.10                  | 0.56  | 175   |
| 5  | 300 mg.        |                                           | 0.11                  | 0.67  | 152   |
| 9  | 300 mg.        |                                           | 0.10                  | 0.52  | 178   |
| 9  | 1 g.           |                                           | 0.10                  | 0.52  | 168   |
| 50 |                |                                           | 0.13                  | 0.62  | 163   |

#### EXAMPLE 5

An emulsion as described in Example 1 is used, except that the test strips after having been exposed, are developed for 8 min. at  $20^\circ$  C. in a developer having the following composition:

Water ( $52^\circ$  C.)—750 ccs.  
N-methyl-p-aminophenol sulphate—2 g.  
Sodium sulphite, anhydrous—100 g.  
60 Hydroquinone—5 g.  
Borax, granular—2 g.  
Water to—1000 ccs.

The sensitometric results are listed in the table hereinafter.

| 70                                                       | Added compound | Amount of compound added per kg. emulsion | Sensitometric results |       |       |
|----------------------------------------------------------|----------------|-------------------------------------------|-----------------------|-------|-------|
|                                                          |                |                                           | Fog                   | Gamma | Speed |
| Polyethylene glycol with average molecular weight 6,000. | 100            |                                           | 0.10                  | 0.48  | 187   |
|                                                          |                | 300 mg.                                   | 0.28                  | 0.58  | 170   |
| 9                                                        | 300 mg.        |                                           | 0.12                  | 0.54  | 168   |
| 9                                                        | 300 mg.        |                                           | Completely fogged     |       |       |

## EXAMPLE 6

A washed negative coarse-grained gelatin silver bromo-iodide emulsion, in which the silver halide consists of 98.2 mole percent of silver bromide and 1.8 mole percent of silver iodide, is ripened at 42° C. After addition of 630 mg. per mole silver halide of 5-methyl-7-hydroxy-s-triazolo[1,5-a] pyrimidine as a stabilizer and other usual ingredients, the emulsion is coated on a support (Sample 1).

Other samples are prepared by adding separately to determined amounts of the same emulsion before coating, the hereafter indicated amounts of developing accelerator. They are then processed in the same manner as Sample 1.

After drying and exposure, the samples are developed for 4 min. in a solution having the following composition:

Water—800 ccs.

Monomethyl-p-aminophenol sulfate—4 g.

Sodium sulfite (anhydrous)—65 g.

Hydroquinone—10 g.

Sodium carbonate (anhydrous)—45 g.

Potassium bromide—5 g.

Water to—1000 ccs.

| Added compound | Amount of compound per kg.<br>emulsion | Sensitometric results |       |       |
|----------------|----------------------------------------|-----------------------|-------|-------|
|                |                                        | Fog                   | Gamma | Speed |
| 2.             | 1 g.                                   | 0.10                  | 1.45  | 85    |
| 2.             | 2.5 g.                                 | 0.13                  | 2.50  | 75    |
|                |                                        | 0.15                  | 2.50  | 66    |

What we claim is:

1. Process for developing photographic materials containing light-sensitive silver halide which comprises the step of developing said materials in the presence of a polymeric compound, containing the following structural units or these units in salt form:



wherein:

each of  $\text{Alk}_1$  and  $\text{Alk}_2$  represent an alkylene group containing from 2 to 10 carbon atoms wherein said chain may contain elements such as oxygen, sulphur, phosphorus, and nitrogen directly linked to two carbon atoms of said alkylene chain,

$\text{R}$  represents an alkyl group of 1 to 5 carbon atoms, a substituted alkyl group, or an aralkyl group,

$\text{R}_1$  represents a hydrogen atom, an alkyl group, a substituted alkyl group or a



5 wherein  $\text{R}_2$  represents an alkyl group, a monovalent unsaturated aliphatic group or a heterocyclic group including said groups in substitution form, and  $n$  is a positive integer of at least 3.

2. Process for developing photographic materials containing light-sensitive silver halide according to claim 1, wherein  $\text{R}_1$  represents a



15 group or its bisulphite addition product.

3. A photographic light-sensitive material comprising a silver halide and a polymeric compound containing the following structural units or these units in salt form:



wherein:

30 each of  $\text{Alk}_1$  and  $\text{Alk}_2$  represent an alkylene group containing from 2 to 10 carbon atoms wherein said chain may contain elements such as oxygen, sulphur, phosphorus, and nitrogen directly linked to two carbon atoms of said alkylene chain,

35  $\text{R}$  represents an alkyl group of 1 to 5 carbon atoms, a substituted alkyl group, or an aralkyl group,

$\text{R}_1$  represents a hydrogen atom, an alkyl group, a substituted alkyl group or a



wherein  $\text{R}_2$  represents an alkyl group, a monovalent unsaturated aliphatic group or a heterocyclic group including said groups in substitution form, and  $n$  is a positive integer of at least 3.

45 4. A photographic light-sensitive silver halide material according to claim 3 containing said polymeric compound in an amount ranging from 100 mg. to 10 g. per mole of silver halide.



## References Cited

## UNITED STATES PATENTS

3,245,793 4/1966 Smith ----- 96—35

NORMAN G. TORCHIN, Primary Examiner

E. C. KIMLIN, Assistant Examiner